

# UNITED STATES PATENT OFFICE.

OSCAR C. M. KNUDSEN, OF BROOKLYN, NEW YORK.

## PROCESS OF PRODUCING A HARD COPPER ALLOY.

1,267,669.

Specification of Letters Patent. Patented May 28, 1918.

No Drawing.

Application filed March 22, 1917. Serial No. 156,744.

*To all whom it may concern:*

Be it known that I, OSCAR C. M. KNUDSEN, a citizen of the United States, residing at Brooklyn, in the county of Kings and State of New York, have invented a new and useful Process of Producing a Hard Copper Alloy, of which the following is a specification.

The present invention relates to a novel process of producing a hard copper alloy, said alloy consisting chiefly of copper and a relatively small percentage of aluminum.

A copper aluminum alloy *per se* is not new, and various methods of uniting them have been employed with some degree of success, but it has been found that by first bringing the aluminum to the melting point, and then placing therein the unmelted copper, and increasing the temperature to or slightly above the melting point of the copper, which is higher than the melting point of aluminum, and thoroughly mixing or stirring the two metals, that a superior product is provided when the alloy cools.

The product can be of varying degrees of hardness, and has been proven by sclerometer tests to possess as high as 68 to 70 per cent. the hardness of tool steel, although the alloy, by changing the proportions of copper and aluminum used, can be of various hardnesses, down to about 45 per cent. the hardness of tool steel. The product, although sufficiently hard, when formed into a lathe tool, to cut steel and other hard metals, is not as brittle and frangible as steel, and is not subject to rusting or corrosion. It has also been proven by tests, that the product of the present process possesses an appreciable degree of elasticity and resiliency,

in addition to its hardness, thus rendering the alloy of advantage for many uses. In fact, the alloy can be used wherever a hard wear and corrosion-resisting metal is desirable. For example, the alloy can be used for propeller shafts to withstand the great strains and conditions to which they are subjected, it not infrequently happening that steel propeller shafts snap and break, resulting in delays and expenses, as well as possible danger to life. The alloy can also be used for the construction of ship hulls to withstand the strains and to prevent the rusting and corrosion of the hulls. For these and many other uses, the alloy will be

particularly advantageous and superior to metals now used, even though the alloy may involve a greater initial expense.

In carrying out the process, from 12 to 14 per cent. of aluminum is used according to the grade of metals used, and according to the degree of hardness desired, the balance of the alloy (from 86 to 88 per cent.) being copper in its pure or commercial form. The aluminum is melted in a crucible, and after being melted has added thereto, the unmelted copper, which is broken up in small particles. The temperature is then increased to or slightly above the melting point of copper, and during the increase in temperature, the particles of copper are thoroughly mixed or stirred with the molten aluminum, whereby as the temperature of the aluminum increases to the melting point of copper, the copper will be thoroughly admixed with the aluminum. It is the addition of the particles of copper in unmelted state with the molten aluminum and the mixing thereof together, which has been found to result in the superior hardening of the alloy when it cools. It has been found that the mixing of the two molten metals together, or the mixing of aluminum with molten copper does not produce the results obtained by the present process. The molten alloy can be cast, rolled, forged or otherwise worked while still hot, and can be used for the production of knives, valves, shafts and various other articles of manufacture.

Having thus described the invention, what is claimed as new is:—

The process of producing a hard alloy composed chiefly of copper and having only a small percentage of aluminum, consisting in melting the aluminum first, then adding thereto the copper broken up into small particles, then increasing the temperature after the copper is added to melt the copper particles, and mixing the copper particles with the molten aluminum during the increased temperature thereof.

In testimony that I claim the foregoing as my own, I have hereto affixed my signature in the presence of two witnesses.

OSCAR C. M. KNUDSEN.

Witnesses:

IVY E. SIMPSON,  
MONROE E. MILLER.